

## UNITED STATES PATENT OFFICE

2,556,241

## SILK SCREEN STENCIL INK

Howard A. Van Etten, Monroe, N. Y., assignor to  
 E. I. du Pont de Nemours & Company, Wil-  
 mington, Del., a corporation of Delaware

No Drawing. Application February 13, 1948,  
 Serial No. 8,272

4 Claims. (Cl. 260—28.5)

1

This invention relates to coating compositions and particularly to coating compositions adapted for application by means of a silk screen stencil and more particularly to those compositions employing vinyl resins.

Silk screen stencil printing is essentially a process in which the stencil bearing the design to be reproduced is permanently affixed to a screen or ground, consisting of silk, organdy, metal cloth, and synthetic fibers, such as nylon, polyethylene, etc.

The process for preparing the stencils consists of applying a coating of a light-sensitive substance adapted to be rendered insoluble upon exposure to light, on a woven web, exposing the light-sensitive coating to light transmitted through a print of the pattern to be reproduced and dissolving and removing the coating from the web not rendered insoluble by light.

Paints, inks or other printing media are forced through that portion of the stencil not coated with the insoluble coating by means of a squeegee and deposited on the surface to be decorated, thus forming a facsimile of the original design. The method is known as the silk screen process because originally silk was exclusively employed for the screen base.

This process has been employed for decorating many surfaces and has been developed to a high state of efficiency. It has been necessary to develop different inks for the various surfaces decorated to insure proper adhesion of the ink to the surface. Recently, polyvinyl chloride and vinyl chloride-acetate copolymer resin coatings have been introduced for a wide variety of uses and have been accepted in view of their superior quality over many other types of coatings formerly used. For many uses the polyvinyl chloride resin coatings require decoration, particularly coated fabrics and unsupported films designed for use as upholstery, tablecloths, novelties, etc. For printing or stenciling polyvinyl chloride resin surfaces, it is desirable to employ inks which contain a polyvinyl chloride resin binder to assure anchorage of the printed design to the base.

The consistency of the composition for satisfactory use as a stencil ink must be such that the material will leave an even, sharply defined surface when dried. It must not be sticky in nature and must break cleanly from the design without stringing when the stencil is removed. For stenciling continuous sheet material, it is necessary that the solvent evaporate before batching the material in roll form. The drying

of the ink is usually carried out by passing the material through a heated tunnel. The rate at which the solvent evaporates from the stencil ink is very important. If the solvent evaporates too rapidly, the stencil will become clogged with partially dried ink. Once a quantity of ink is placed on a stencil screen, it should not change in either its consistency or its property to break away sharply from the stencil when the stencil is removed from the surface being decorated.

It is an object of this invention to provide a vinyl resin stencil ink for use in decorating vinyl resin coated fabrics. A further object is to provide a vinyl resin stencil ink which will permit the screen to release readily from the surface being decorated and not form "legs" or develop stringiness when the stencil is pulled away from the surface being stenciled. A still further object is to provide a vinyl resin stencil ink which will not change in consistency when being moved back and forth across a silk screen stencil by means of a squeegee in a continuous stencil operation. Other important objects will be readily apparent as the description of the invention proceeds.

The objects of this invention are accomplished by incorporation of wax into a composition comprising a soluble vinyl resin, pigment, solvent and a plasticizer, in which the pigment is present in amounts of from 60% to 80% of the non-volatile ingredients in the composition.

In the claims the term "soluble polyvinyl chloride resin" is used to describe the copolymer resins which are sufficiently soluble in methyl ethyl ketone that a 20-25% solution in methyl ethyl ketone at room temperature will form a free flowing liquid.

The following detailed examples are given by way of illustration and not limitation, in which the percentage figures are all given on a weight basis.

## Example I

A red stencil ink was prepared by first dissolving the vinyl resin binder in hot methyl ethyl ketone as per the following formula:

|                              | Per cent |
|------------------------------|----------|
| Polyvinyl resin <sup>1</sup> | 25       |
| Methyl ethyl ketone          | 75       |

<sup>1</sup> The polyvinyl resin used in this example was a multi-polymer, the approximate composition of which may vary within the following limits:

80% to 90% by weight of combined vinyl chloride, 19.7% to 7.0% by weight of combined vinyl acetate, 0.3% to 3.0% by weight of maleic or similar alpha-beta olefinic unsaturated carboxylic acid.

The following ingredients were premixed before grinding on a three roll paint mill:

|                                                            | Wet      | Dry      |
|------------------------------------------------------------|----------|----------|
|                                                            | Per cent | Per cent |
| 25% solution polyvinyl resin in methyl ethyl ketone, supra | 36.80    | 15.40    |
| Cadmium sulfide—red pigment                                | 43.20    | 72.00    |
| Polypropylene glycol sebacate                              | 6.38     | 10.60    |
| Methyl ethyl ketone                                        | 9.82     |          |
| 20% dispersion of paraffin wax in toluol                   | 3.20     | 1.00     |
| Malic acid                                                 | .69      | 1.00     |
|                                                            | 100.00   | 100.00   |

The stencil ink was employed for the decoration of tablecloth material comprising a fabric base coated with a polyvinyl chloride resin composition. The ink was applied to the coated fabric by the silk screen process described above. A final surface coat of clear unpigmented solution of a polyvinyl chloride resin was applied over the entire surface of the fabric coating. The preparation of the coated fabric and the stenciling operation was carried out in the manner described by Howard Van Etten in an application filed July 3, 1946, Serial No. 681,407 now Patent No. 2,453,052.

#### Example II

A stencil ink was prepared using a resin different from that disclosed in Example I, as indicated below:

|                                                                                 | Per cent |
|---------------------------------------------------------------------------------|----------|
| Copolymer of vinyl chloride and vinyl acetate in the approximate ratio of 85:15 | 20       |
| Ethyl acetate                                                                   | 80       |

A suitable copolymer resin for use in this example may be obtained on the open market under the trade name of "Vinylite" VYHH, which is sold by Carbide & Carbon Chemicals Corporation.

The following ingredients were thoroughly mixed before grinding on a three roll paint mill:

|                                                                                             | Wet      | Dry      |
|---------------------------------------------------------------------------------------------|----------|----------|
|                                                                                             | Per cent | Per cent |
| 20% solution of copolymer of 85 vinyl chloride and 15 vinyl acetate in ethyl acetate, supra | 35.80    | 15.10    |
| Cadmium sulfide—red pigment                                                                 | 34.60    | 72.00    |
| Polypropylene glycol sebacate                                                               | 5.40     | 11.10    |
| Methyl ethyl ketone                                                                         | 8.00     |          |
| 20% dispersion of paraffin wax in toluol                                                    | 2.70     | 1.00     |
| Ethyl acetate                                                                               | 13.50    |          |
|                                                                                             | 100.00   | 100.00   |

#### Example III

A blue stencil ink was prepared as follows:

|                                                                             | Per cent |
|-----------------------------------------------------------------------------|----------|
| 25% solution of vinyl resin referred to in Example I in methyl ethyl ketone | 36.6     |
| Blue pigment-copper phthalocyanine                                          | 3.9      |
| Barytes                                                                     | 40.0     |
| Diocetyl phthalate                                                          | 6.5      |
| Malic acid                                                                  | 1.0      |
| Methyl ethyl ketone                                                         | 9.7      |
| 20% dispersion of paraffin wax in toluol                                    | 3.2      |

A complete breakdown of the above is as follows:

|                                                    | Wet      | Dry      |
|----------------------------------------------------|----------|----------|
|                                                    | Per cent | Per cent |
| Polyvinyl chloride-vinyl acetate-maleic acid resin | 9.15     | 15.18    |
| Diocetyl phthalate                                 | 6.50     | 10.75    |
| Blue pigment-copper phthalocyanine                 | 3.00     | 4.98     |
| Barytes                                            | 40.00    | 66.37    |
| Malic acid                                         | 1.00     | 1.66     |
| Paraffin wax                                       | .64      | 1.06     |
| Toluol                                             | 2.56     |          |
| Methyl ethyl ketone                                | 37.15    |          |

The stencil ink of this example was prepared in the same manner as described in Example I.

The stencil inks of Examples II and III were employed for decorating polyvinyl chloride coated fabric as described in Example I. The designs formed had sharp definition, and there was substantially no tendency for the silk screen to adhere to the surface being decorated when it was pulled away. Also, there was little or no tendency for the ink to thicken and clog the silk screen stencil interstices through which the ink is forced by means of a squeegee.

Compositions having the same formulae as those described in Examples I, II and III, except that the paraffin wax was omitted, were prepared and employed as stencil inks for polyvinyl chloride resin coated fabric in the manner described above. The silk screen could not be readily separated from the surface being decorated and the ink formed "legs" when the silk screen was pulled away and did not form a clean-cut and well defined design. Also, the ink clogged part of the openings in the silk screen stencil after it was drawn back and forth over the screen by a squeegee a relatively few times.

The vinyl resin for use in practicing this invention must be sufficiently soluble in relatively low boiling solvents, such as, e. g., methyl ethyl ketone, that a 20-25% solution will form a free flowing liquid at room temperature. The copolymers of vinyl chloride with vinyl acetate, ethyl fumarate, vinylidene chloride, etc. are satisfactory, particularly where the vinyl chloride represents 80-90% of the polymer. As indicated in Example I, such copolymer resins may be modified with a small amount of polycarboxylic acid.

It will be noted that in Example II the resin is first dispersed in ethyl acetate which does not have as great a solvent action on the resin as methyl ethyl ketone. This results in a composition which is somewhat "short" or apple saucy. This is an advantage and represents the preferred embodiment since the inks made with the resin dispersed in ethyl acetate are of a mayonnaise consistency and have less tendency to flow around the edges of the squeegee during application and also less tendency to leak through the openings in the stencil screen unless pressure is applied.

There is considerable latitude in choice of pigments for this invention. In the case of solutions of the vinyl chloride vinyl acetate-maleic acid multipolymer, the presence of unreacted carboxyl groups results in a tendency toward reactivity with basic pigments which results in gelling of the solution. This gelling is overcome or prevented by the presence of small amounts of acidic or basic substances. The use of malic acid together with other organic acids with dispersions of multipolymer of vinyl chloride, vinyl acetate and maleic acid in the presence of basic pigments to prevent gelation is disclosed and claimed in copending application Serial No. 770,195, filed August 22, 1947, by H. T. Doderer, now abandoned.

Where stain resistance is required for certain application of the coating, such as, e. g., tablecloths, wall coverings, aprons, etc.; a non-migrating type of plasticizer, such as polypropylene glycol sebacate and polypropylene glycol adipate, as well as other polyesters, is required, since it has less affinity for various stains. Where stain resistance is not important, other plasticizers of the monomeric ester type may be used, such as,

e. g., dioctyl phthalate, tricresyl phosphate, dibutoxy ethyl phthalate, dibutoxy ethyl sebacate, etc.

In order to obtain sufficient coverage of the base coating in one application of the stencil ink, the pigment content should not be less than 60% of the total solids of the ink. The maximum amount of pigment which can be employed is 80% of the total solids. The specific choice of pigment will determine the preferred amount, since oil absorption, covering power, effect on film strength, etc., vary with different pigments. The ratio of pigment to binder and plasticizer in the composition of this invention is considerably higher than normally employed for coating compositions.

The high percentage of pigments in the stencil paste of this invention does not permit the composition to be prepared by conventional methods, such as, e. g., dissolving the binder in an organic solvent, separately grinding the pigments in plasticizer, then combining the binder solution with the pigment-plasticizer mixture. Due to the low ratio of liquid ingredients to the pigment, it is necessary to first dissolve the binder in an organic solvent, then add the dry pigment and plasticizer to the binder solution, after which the entire composition is ground on a three roll paint mill. In practice the stencil inks of this invention are usually coated over with a clear (non-pigmented) solution of vinyl resin to prevent the pigment particles from being abraded off in service.

As indicated above the presence of a small amount of a wax is essential in the composition of this invention. Inks containing as little as 0.5% of wax and those containing as high as 5% based on the total non-volatile content of the ink have been found useful. Approximately 1%, based on the non-volatile content, is the preferred amount of wax. Paraffin wax is preferred due to its solubility in volatile organic solvents.

The compositions of this invention are designed specifically for application by means of a silk screen stencil. They are also useful as printing inks for application by means of intaglio print rollers. For application by means of intaglio print rolls the compositions described in the examples should preferably be diluted somewhat with the volatile solvent.

It is apparent that many widely different embodiments of this invention may be made without departing from the spirit and scope thereof, and therefore, it is not intended to be limited except as indicated in the appended claims.

I claim:

1. A stencil ink having the following composition by weight:

Per cent

|                                                                                 |        |
|---------------------------------------------------------------------------------|--------|
| 25% solution of a copolymer of 85% polyvinyl chloride and 15% polyvinyl acetate | 35.80  |
| 5 Pigment                                                                       | 34.60  |
| Polypropylene glycol sebacate                                                   | 5.40   |
| Methyl ethyl ketone                                                             | 8.00   |
| 20% dispersion of paraffin wax in toluol                                        | 2.70   |
| Ethyl acetate                                                                   | 13.50  |
|                                                                                 | 100.00 |

10  
15  
15. A stencil ink of claim 4 consisting essentially of a polyvinyl chloride-polyvinyl acetate-maleic acid resin, 1% maleic acid, from 60 to 80% pigment, from 0.5% to 5.0% wax all based on the non-volatile content of the ink.

20  
20. The product of claim 4 in which the polyvinyl resin is a copolymer prepared by polymerizing a monomeric mixture containing 85% vinyl chloride and 15% vinyl acetate.

25  
25. A stencil ink comprising a vinyl resin, plasticizer, wax, pigment and a mixture of volatile solvents for the said resin and wax, the said pigment being present in amount between 60% and 80%, the wax being present in amount between 0.5% and 5.0% both based on the weight of the non-volatile components of the ink, the balance of the non-volatile portion being a resin polymerized from a mixture of 80% to 90% vinyl chloride, up to 3% of maleic acid and the balance being vinyl acetate, a 20% to 25% solution of the resin in methyl ethyl ketone being free-flowing liquid at room temperature.

30  
35  
35. HOWARD A. VAN ETEN.

#### REFERENCES CITED

The following references are of record in the file of this patent:

#### UNITED STATES PATENTS

| Number    | Name          | Date          |
|-----------|---------------|---------------|
| 2,073,229 | Shuey         | Mar. 9, 1937  |
| 2,254,072 | Jenkins       | Aug. 26, 1941 |
| 2,264,625 | Doolittle     | Dec. 2, 1941  |
| 2,268,595 | Huber et al.  | Jan. 6, 1942  |
| 2,391,621 | Powell et al. | Dec. 25, 1945 |

#### OTHER REFERENCES

- Fligor et al.: Ind. and Eng. Chem., vol. 37, No. 50 5, May 1945 (pp. 504-508).  
 Ellis: Printing Inks (Reinhold Pub. Co.), 1940, page 116.  
 Wolfe: Printing and Litho Inks (MacNair-Dorland), 3rd ed., 1941, page 291.  
 55 Pollack: Plastics, January 1946, pp. 35-38 and 123.